

## UNITED STATES PATENT OFFICE

SHELDON B. HEATH, OF MIDLAND, MICHIGAN, ASSIGNOR TO THE DOW CHEMICAL COMPANY, OF MIDLAND, MICHIGAN, A CORPORATION OF MICHIGAN

## METHOD OF MAKING METALLIC MAGNESIUM

No Drawing.

Application filed May 25, 1928. Serial No. 280,659.

The present invention concerns a method of producing metallic magnesium by the electrolysis of a fused bath containing magnesium chloride ( $MgCl_2$ ) and concerns more particularly the method of maintaining the bath by feeding to it a compound of magnesium.

In the electrolysis of such a fused bath wherein metallic magnesium is liberated and collects at the cathode and chlorine is liberated and drawn off at the anode, continuous operation is desirable and it becomes necessary to replenish the bath and maintain it of the desired character by feeding thereto an equivalent of the magnesium and chlorine or other essential ingredients which, in the course of operation, have been or may be removed therefrom.

It is well known that the ideal feed to such a cell comprises anhydrous  $MgCl_2$  and that accompanying water will reduce the current and power efficiency of electrolysis. It is further known that inert constituents of the feed, such as  $MgO$ , tend to settle out of the bath, and unless removed therefrom, will accumulate and interfere with continuous operation. Such sediment must accordingly be removed, which is customarily done by dipping from time to time as required, but this operation removes also part of the bath along with the sediment or so-called sludge. In practice I have found that as high as two equivalents of  $MgCl_2$  may be removed in that way with one equivalent of sludge figured as  $MgO$ . The bath so removed with the sludge must, of course, be returned by feeding to the cell the constituents removed in addition to that required to replenish the  $MgCl_2$  converted to metal and chlorine.

Anhydrous  $MgCl_2$  is not only difficult and expensive to prepare, but on account of its hygroscopic properties it is practically impossible to handle it without its taking up some moisture, and in practice, a content of 95%  $MgCl_2$  in the chloride fed to the cell is considered obtainable good practice.

In U. S. Patent No. 1,567,318 is disclosed a method of feeding  $MgCl_2$  containing water, whereby the detrimental effects of the water are minimized.

I have discovered an improved method of introducing the  $MgCl_2$  fed to such an electrolytic cell, having advantages as contrasted with the method therein disclosed, said improved method of feeding involving broadly the introduction of  $MgCl_2$  containing basic salt, such as magnesium oxy-chloride ( $MgOHCl$ ).

To the accomplishment of the foregoing and related ends, the invention, then, consists of the steps hereinafter fully described and particularly pointed out in the claim, the following description setting forth in detail one approved method of carrying out my invention.

I have found that when  $MgCl_2$ , containing water is introduced into a fused bath containing  $MgCl_2$ , such as may be used in an electrolytic cell for the production of metallic magnesium and chlorine, decomposition occurs consuming the heat of the cell and bath to form gaseous products containing  $HCl$  and basic salt corresponding to a portion of the accompanying water. Such basic salt I find corresponds to the oxy-chloride ( $MgOHCl$ ).

I have found that instead of feeding such  $MgCl_2$  containing water it is more advantageous to further dehydrate with cheaper heat than that available in an electrolytic cell to form  $MgCl_2$  containing a portion of the basic salt corresponding to  $MgOHCl$  and to feed that product to the cell as the source of  $MgCl_2$  therefor. Such a product enters into the bath without decomposition.

In the patent cited above there is disclosed and claimed the method of feeding magnesium chloride adjacent the anode, but I have found that magnesium chloride containing small quantities of basic salt may be fed adjacent the cathode or through the neutral zone if the cell be of a type providing such a zone. I have found that  $MgCl_2$  containing as high as 5% equivalent  $MgOHCl$  may be fed to either anode or cathode or neutral zone. If the content of basic chloride be in excess of 5% I prefer, however, to feed it adjacent the anode.

Magnesium chloride prepared as  $MgCl_2$  anhydrous containing a small amount of basic chloride is an intermediate product in

the preparation of a strictly anhydrous chloride according to certain methods of procedure and is therefore a cheaper source of magnesium than is the still further processed anhydrous material.

When hydrated magnesium chloride is dried, either in air, wet or dry, or in any inert atmosphere, whether at reduced pressure or in vacuum until all water as such together with hydrochloric acid is driven off, there results a product containing magnesium, chlorine, oxygen and hydrogen. A peculiarity of this product is that if the hydrogen content be figured as water ( $H_2O$ ) and the remaining oxygen be figured as magnesium oxide  $MgO$ , the molecular ratio of the latter to the former is constant at unity, no matter what the total content of such hydrogen and oxygen may be, it being understood that such total content will vary depending upon the method and rate of drying. This it is believed indicates that the product in question is comprised of magnesium chloride ( $MgCl_2$ ), anhydrous, and the oxychloride ( $MgOHCl$ ). For want of a better term, this product is hence referred to as magnesium chloride containing basic magnesium chloride; however, it is not intended thereby to define the product to one having any precise constitutional formula.

If desired, the aforesaid product may be fed to the cell in molten condition, and thereby conserve the heat of the cell.

It should be noted further that, in practice, other additive constituents or constituent of the bath such as  $NaCl$  or  $NaF$  may be desirably used, and such will be removed along with the magnesium constituent with the dipped sludge. Depletion of such constituents or constituent if so or otherwise removed will necessarily require a corresponding amount to be added to maintain the bath of the desired composition and such addition may conveniently be made along with the feed of the magnesium salt used.

Other modes of applying the principle of my invention may be employed instead of the one explained, change being made as regards the method herein disclosed, provided the step or steps stated by the following claim or the equivalent of such stated step or steps be employed.

I therefore particularly point out and distinctly claim as my invention:—

55 In a method of producing metallic magnesium, including the electrolysis of a fused bath containing magnesium chloride, the step which consists in maintaining said bath by introducing adjacent the anode magnesium chloride containing in excess of five per cent. of basic magnesium chloride.

Signed by me this 14 day of May, 1928.  
SHELDON B. HEATH.